

April 10, 1951

C. M. ANDERSON ET AL

2,548,187

METHOD OF DETERMINING THE OXYGEN CONTENT OF COPPER

Filed July 19, 1945



INVENTORS

C. M. ANDERSON  
R. A. HARRIS  
C. C. PATTON

BY Harry L. Duff  
ATTORNEY

## UNITED STATES PATENT OFFICE

2,548,187

METHOD OF DETERMINING THE OXYGEN  
CONTENT OF COPPER

Carl M. Anderson, Chicago, Robert A. Harris, Oak Park, and Charles C. Patton, Chicago, Ill., assignors to Western Electric Company, Incorporated, New York, N. Y., a corporation of New York

Application July 19, 1945, Serial No. 605,950

3 Claims. (Cl. 23—230)

1

This invention relates to a method of determining the oxygen content of copper.

In the manufacture of some articles from copper, it becomes necessary to braze or treat the articles in a reducing atmosphere as a step incident to the manufacture of the articles. In such articles, the presence of even very small quantities of oxygen in the copper cause warping of the copper parts and, as a consequence of this distortion, the articles are defective. Accordingly, it has become of primary importance to determine the purity of copper to be used in such processes.

It is an object of the present invention to provide a method of determining oxygen in the copper.

In accordance with one embodiment of the invention, a sample of copper is heated in a hydrogen atmosphere or a reducing atmosphere containing a relatively large amount of hydrogen and then cooled in the same atmosphere. Prior to heating the sample, it is measured to determine its diameter and, after the heating and cooling in the reducing atmosphere, it is again measured. It has been found that copper containing oxygen will grow when heated to elevated temperatures in the presence of hydrogen, apparently due to the formation of voids at the grain boundaries when the oxygen and hydrogen combine.

A complete understanding of the invention may be had by reference to the following detailed description when considered in conjunction with the accompanying drawing, wherein the single figure illustrates graphically the percent of increase in diameter of various commercial brands of pure copper when treated in accordance with the present invention.

Commercial electrolytic copper, known as tough pitch copper, is known to contain from approximately .03% to approximately .05% of cuprous oxide and for most manufacturing purposes, where a high degree of conductivity is required, copper containing a maximum of .07% of oxygen is acceptable. However, in the manufacture of some parts which are later to be treated in a reducing atmosphere, the amount of oxygen in commercially pure or electrolytic copper is too great and the parts to be manufactured become embrittled and warped, whereas the material known as "oxygen-free high conductivity copper" is sufficiently low in its oxygen content so that no deleterious embrittlement or warping will occur when parts made from this material are treated in reducing atmospheres.

2

In accordance with the present invention, copper rods of from as small as .25" in diameter to as large as approximately .8" in diameter and just under one inch long are heated to an elevated temperature in the presence of either pure hydrogen or a gas such as "ammo" gas containing 75% H<sub>2</sub>, 25% N at temperatures from 1550° F. to 1850° F. and then are cooled in the same atmosphere, whereupon a comparison of the diameter of the samples prior to and after heat treating will indicate whether or not there is oxygen in the samples. In accordance with the present invention, the samples are held at the selected temperature for from fifteen to twenty minutes and then are cooled while in the same atmosphere. Since it is known that cuprous oxide goes into solution in melted copper and tends to go out of solution in solid copper and, further, that cuprous oxide apparently, upon the cooling of the copper, tends to accumulate along the grain boundaries of the copper, it is believed that the hydrogen from the controlled atmosphere in the heat treating furnace combines with the oxides at the grain boundaries and probably some of it escapes as steam, leaving voids at the boundaries. The combining of the hydrogen and oxygen at these high temperatures will form steam which requires more space than the oxides, thus leaving the voids and increasing the overall dimensions of the sample.

Examination of copper treated in this manner when a microsection is examined at a suitable magnification, such as 75X, shows voids at the grain boundaries, which probably accounts for the dimensional growth of the samples. It has been further noticed in the course of experiments that the diameter of a rod exhibits a much greater tendency to grow than a comparable length of rod. This apparently has resulted from the distortion of the grain structure in the formation of the rod, thus providing more boundaries in the cross-sectional area of the rod for a given dimension than in the length of the rod for the same dimension. As indicated in the drawing, a number of samples of commercially pure copper have been tested and seem to clearly exhibit that the heat treatment described hereinbefore will cause a measurable change in physical dimensions of copper samples which is dependent upon the amount of oxygen in the copper. In the experiments conducted in perfecting the present invention, samples of tough pitch copper, phosphorous deoxidized copper, phosphorous deoxidized copper containing a small amount of tellurium, and the product known as

"oxygen-free high conductivity copper" were tested. The samples tested indicated that growth occurs when there is oxygen present in the samples.

As indicated in the drawing, the percent increase in diameter of tough pitch copper, when treated at temperatures ranging from 1550° F. to 1850° F. in atmospheres containing principally hydrogen, gradually increases from approximately 1.29% to approximately 2.04%. This apparently indicates that as the treating temperature is raised, the amount of expansion or growth of the sample increases progressively. However, there is a limit to the temperature which may be used since somewhere just above 1850° F. the copper becomes so plastic as it approaches the molten stage that the measurement of it would not be accurate. The samples of tough pitch copper tested were approximately  $\frac{1}{2}$ " in diameter and almost one inch in length and their growth in diameter followed the line 1.

A number of phosphorous deoxidized copper samples having some tellurium in them were tested under the same temperature and atmospheric conditions and they exhibited a growth from where their percentage of increase in diameter, after heat treatment and cooling, ranged from .458% at 1550° F. to 1.65% at 1850° F., as indicated by the line 2. A number of samples of "oxygen-free high conductivity copper" containing a small amount of tellurium changed in diameter from an increase of from .04% at 1550° F. to a maximum of .128% at 1850° F., as indicated by the line 5.

In tests where the same conditions were maintained, a number of samples of "oxygen-free high conductivity copper" treated at 1550° F., 1607° F., 1650° F., 1750° F., and 1850° F. were measured and three of the samples, as indicated by the encircled dots at 3, apparently shrank, whereas four samples, as indicated by the encircled dots 4, apparently maintained exactly the same diameter. This is believed to indicate that the "oxygen-free high conductivity copper" did not grow in size and, inasmuch as the three samples which apparently shrank are within the range of accuracy of the measurements made, it is safe to assume that there will be no change in size of copper samples which are free from oxygen when the copper is treated at the elevated temperatures in a hydrogen atmosphere and it is also believed to be fair to assume that a small amount of oxygen in copper will cause the copper to increase in size when treated as described hereinbefore. When the copper increases in diameter less than .20%, it is acceptable and does not warp or become embrittled to a detectable extent when used in the manu-

facture of electrical apparatus which is later treated in a hydrogen atmosphere.

What is claimed is:

1. The method of determining the deleterious effect of the oxygen content of copper which comprises determining the dimensions of a sample of copper, heating said sample to from approximately 1550° F. to approximately 1850° F. for from fifteen to twenty minutes, cooling the sample to room temperature, maintaining a hydrogen atmosphere around the sample during the heating and cooling, and then again determining said dimensions to indicate variations in said measurement above and below .20% of the original dimensions.

2. The method of grading various samples of coppers in cylindrical form by determining the deleterious effect of the oxygen content in each sample, which comprises determining the diameter of each sample of copper, heating each sample to from approximately 1550° F. to approximately 1850° F. for from fifteen to twenty minutes, cooling each sample to room temperature, maintaining a hydrogen atmosphere around each sample during the heating and cooling, and then again determining said diameters to ascertain whether the percent increase in diameter for each sample falls below a predetermined value.

3. The method of grading coppers by determining the deleterious effect of the oxygen content in various samples of the coppers, which comprises determining a particular dimension of each sample of copper, heating each of said samples to a predetermined temperature within the range of 1550° F. to approximately 1850° F. for from fifteen to twenty minutes, cooling each sample to room temperature, maintaining a reducing atmosphere containing hydrogen around each sample during the heating and cooling, and then again determining said dimension of each individual sample to ascertain the percent change in size relative to a predetermined value to determine the grading of each sample.

CARL M. ANDERSON.

ROBERT A. HARRIS.

CHARLES C. PATTON.

#### REFERENCES CITED

The following references are of record in the file of this patent:

N. B. Pilling, "Action of Reducing Gases on Hot Solid Copper," Trans. A. I. M. E. 1919, vol. 60, p. 322.

Metals Handbook, American Society for Metals, 1939, Cleveland, Ohio, p. 1391.

Rhines et al., Trans. A. I. M. E., vol. 143, 1941, pages 312-325.